

June 17, 1941.

K. SCHINZEL ET AL

2,246,013

COLOR SOUND FILM

Filed June 18, 1938



Inventors

Karl Schinzel  
Ludwig Schinzel

By

Newton M. Perkins  
R. Frank Smith

Attorneys

## UNITED STATES PATENT OFFICE

2,246,013

## COLOR SOUND FILM

Karl Schinzel, Rochester, N. Y., and Ludwig Schinzel, Troppau, Silesia; said Karl Schinzel assignor to Eastman Kodak Company, Rochester, N. Y., a corporation of New Jersey

Application June 18, 1938, Serial No. 214,578  
In Austria June 25, 1937

2 Claims. (Cl. 95—2)

This invention relates to photographic color films having sound images therein, and to methods of producing such films.

Development of a sound film to a certain gamma is only a poor compromise. It would be ideal, if the sound track and the image could be developed entirely independent of each other. In the accompanying drawing, the figure is a flow diagram showing sectional views of successive steps in one method of forming a sound track image according to our invention.

On thin single emulsions drying very rapidly, this may be realized by developing first only the scenes or the sound track to the desired density, using anti-fogging agents, for example, nitrobenzimidazole and other azimides, tri- and tetrazoles, thiosemicarbazones. The film is then dried and the other image printed, developed, etc. Variable width recording should be printed and developed before the scenes. Very thin and weakly tanned emulsions do not have to be dried, and the next image may be printed immediately after development and washing of the first image. Addition of anti-fogging agents is necessary in the second development.

Double emulsions or those having differently sensitized zones are superior, the scenes being in one emulsion layer or zone and the sound track in the other one, nearest the support. Thin emulsion layers must be used to shorten the drying time. The emulsion for the variable width recording may be much thinner and harder than that for the scenes, which should be softer and perhaps more sensitive or contain more silver halide. The two emulsion layers are separated from each other by an easily decolorized yellow filter layer and printed from different sides. The color sensitivity of the emulsion layers may also be different, one for blue-green or yellow, and the other for red or infrared, and they are printed with the corresponding light. Ultraviolet light should be used for printing the variable width record on a fine-grain or grainless emulsion. A yellow or colorless ultraviolet-absorbing intermediate layer must then be present, and the original sound record must be on material which is opaque to ultraviolet rays, for example, on copper ferrocyanide. X-rays may also be used for printing, if the silver halide of the sound track emulsion has been sensitized with the thorium salt of eosin, and the original is transparent to X-rays. The variable width sound record should be printed and developed before the scenes. If the emulsion for the scenes is sufficiently sensitive, it may also be used for direct

taking of the scenes, and the sound record exposed or printed simultaneously or later on the negative for which also ultraviolet rays or a cathode ray oscilloscope may be used.

5 The lower emulsion may be tanned or consist of hardened gelatin, and the upper emulsion of soft gelatin. After the image in the upper emulsion is developed and fixed, the sound track in the lower emulsion layer is developed for a longer time and in a slightly warmed developer or after destruction of the tanning effect. This lower emulsion layer may also consist of silver halide collodion emulsion which may have been hardened before coating the upper emulsion layer to make it more difficultly developable. Both emulsion layers must, of course, be differently sensitized, or separated from each other by a filter layer, or even dyed, and they are printed from both sides.

10 20 A light-sensitive substance, which is not attacked by the developer required for the other emulsion layer, is used for the sound track. The lower emulsion layer, consisting of gelatin, collodion, etc., may also contain leuco bases, insoluble or at least not noticeably diffusing salts of indigosols, thioindigosols or similar leuco esters, also black or any other colored or colorless substances which do not react during development of the upper emulsion layer containing the image, and are also unaffected by hypo, as for example, o-nitrobenzaldehyde, diazo sulfonic acids and diazo anhydrides with or without the necessary components. The sound track is now printed to the desired density from the original or its copy

15 25 30 35 40 45 50

which must be opaque to ultraviolet, using the strong ultraviolet rays of a mercury quartz lamp. Finally, the unused bases are washed out in dilute monochloracetic acid, salts of indigosols with cinchonine, triphenylguanidine, diphenylguanidine, etc., in dilute solutions of sodium carbonate, ammonia or sodium hydroxide which may have to be prepared with alcohol. Unused anhydride is coupled to itself or to the component in ammonia vapors, dilute alcoholic sodium hydroxide, or ammonia; or vapors or solutions of acetone and ammonia are allowed to react on the residual o-nitrobenzaldehyde. The light-sensitive substance for the sound track may also consist of mercuric bromide or other organic salts, and the residue may be blackened after development and fixing with sodium sulfide. Emulsions of slight sensitivity of the Lippmann type which may be sensitized may also be physically developed by the Goldberg or Odell methods, but the sound track must be printed corre-

spondingly longer. Although the scenes developed previously are intensified by this procedure, this effect may be lessened without harm to the film by wiping the film off after protecting the sound track.

Two different silver halide emulsions are used in which the silver halide of one emulsion layer is more easily developed than that of the other layer. Among the possible combinations are AgCl—AgBr, AgCl—AgI, AgBr—AgI. The first one appears to be the best adapted, since silver chloride is much more easily reduced by certain developers than silver bromide. For printing, however, mercuric bromide, silver iodide, and especially silver ferrocyanide, are better suited, because they are much less attacked than silver ferrocyanide, but they cannot, or only to a limited degree, be made color sensitive. If a lower silver iodide emulsion layer is combined with a soft upper silver bromide emulsion sensitized with erythrosine, and both are separated from each other by an easily decolorized yellow filter or are temporarily colored yellow, the scenes are developed first in the upper emulsion layer with a weak developer, the residual silver bromide immediately fixed out, and then the sound track developed in the lower silver iodide emulsion with a strong developer and fixed.

A 1% sodium quinone sulfonate solution and 5% anhydrous sodium sulfite (hydroquinonedisulfonic acid) develops an image on silver chloride gelatin in a few minutes, but it does not affect overexposed silver bromide after half an hour's development. Hydroquinone, pyrocatechin, pyrogallol, amidol, and numerous other developing substances behave similarly under certain conditions which are described in detail in the literature also several simple and compound color developers (Schinzel patent application S. N. 139,758). This difference of developability is less striking in silver chloro-bromide emulsions.

If the original triple-emulsion, however, consists of silver chloride, a fourth lower silver bromide emulsion may be arranged for the sound track. A film of this type is illustrated in the first stage of the figure of the accompanying drawing in which 10 is a suitable transparent support coated with a silver halide layer 11 of soft gelatin for recording the sound track, and silver halide layers 13, 14 and 15 sensitive respectively to the red, green and blue regions of the spectrum and consisting of hard gelatin, all of these layers being separated from the soft gelatin layer 11 by a yellow or ultra-violet filter layer 12. The picture area of the film is exposed from the emulsion side to form latent images in the hard gelatin layers and since the film contains the filter layer 12 these images are not recorded on the layer 11 which is sensitive only to blue light. After exposing or printing of the three separation images on the silver chloride gelatin emulsions, the exposed picture areas may then be developed, as shown in the second stage of the figure to form images 16, 17 and 18 in the layers 13, 14 and 15, respectively, the sound track alone being printed dry and through the back on the correspondingly sensitized silver bromide emulsion or on one protected by filters. This emulsion layer is sensitized for infrared or separated from the triple-emulsion by an ultraviolet-absorbing filter, according to whether infrared or ultraviolet-light is used for printing. If the picture areas have not been already developed they may be then first developed with qui-

none sulfonic acid and sodium sulfite on the places of the residual silver chloride, coupled with the components in the three-emulsion layers by means of p-aminodimethyl-aniline, and the sound track developed simultaneously, or if the picture areas have already been developed the exposed soft gelatin layer 11 may be developed to form a metallic silver sound image 19, then all reduced silver converted into silver ferrocyanide, the residual silver bromide developed and finally fixed. This leaves dye images 16, 17, and 18 in layers 13, 14, and 15 and sound image 19 in layer 11, as shown in the third stage of the figure. In a variation, one may develop the residual silver bromide to any dye and remove all silver simultaneously with Farmer's reducer.

It is, of course, understood that in all materials mentioned in this description anti-halation layers must be used, so that very sharp sound records and prints may be obtained.

It is sometimes of advantage to combine some of the methods described with "controlled diffusion." The action may be limited to the outermost layer or zone, if alcoholic solutions of developers or other reagents containing only a few per cents of water are used, so that an independent development of the sound record is guaranteed. Oxidizing agents may also be used in this form for the reduced silver of both emulsions, and oxidize only the silver in the upper emulsion, or convert it into other compounds which may later be dissolved by water or hypo. It is, of course, assumed that the emulsion intended for the sound track is on top, if such a treatment is considered; in this case, it may be necessary to expose through the back.

In the examples given in the present description of printing three-color images with or without sound track, as well as in analogous printing processes with colored development and coupling, it is often desirable to reproduce black as a color or as silver instead of the subtractive method of superposition of three dyes, if necessary, for the separation image. This black separation image can be produced relatively simply by processes based on colored development and coupling, where the entire silver is still present at the end in the triple or single emulsion. It is only necessary to rehalogenate or to sensitize. The black silver is developed and fixed or converted to a black dye, and the silver thoroughly removed with Farmer's solution. In the oxidation methods mentioned in this description, the matter is simple only when silver salts or metallic silver is still present which may easily be converted into sensitive silver halide or perhaps silver ferrocyanide, after which the procedure is the same as just outlined. Otherwise, one is obliged to obtain an insoluble silver halide or silver ferrocyanide by conversion with a silver salt solution, or to impregnate with light-sensitive salts, or to precipitate a silver halide diffusely through the entire emulsion and to obtain the black image by exposure and development, also colored development, and fixing.

What we claim is:

1. The method of printing the sound track image and picture image on multi-layer photographic material having at least two sensitive layers, an upper layer being composed of soft gelatin containing sensitive silver chloride and a lower layer being composed of harder gelatin containing sensitive silver bromide, which comprises printing the picture image in the layer of soft gelatin, developing it in a weak developer

and fixing out the residual silver chloride, and then printing the sound track image in the layer of harder gelatin, developing it in a strong developer and fixing it.

2. The method of printing a sound track image and a picture image on multi-layer photographic material having at least one light-sensitive layer of gelatino-silver chloride and at least one light-sensitive layer of gelatino-silver bromide, which comprises printing the sound track image on a 10

5 gelatino-silver bromide layer and the picture image on at least one of the gelatino-silver chloride layers, developing the picture image in a sodium quinone sulfonate and sodium sulfite developer and then developing the gelatino-silver bromide layer in a developer selected from the group consisting of hydroquinone, pyrocatechin, pyrogallol and amidol.

KARL SCHINZEL.  
LUDWIG SCHINZEL.